

Patented June 14, 1938

2,120,244

# UNITED STATES PATENT OFFICE

2,120,244

## TREATMENT OF MOTOR FUEL

Charles G. Dryer, Chicago, Ill., assignor to Universal Oil Products Company, Chicago, Ill., a corporation of Delaware

No Drawing. Application August 31, 1935,  
Serial No. 38,793

16 Claims.

(Cl. 44—9)

This invention relates to the treatment of hydrocarbon motor fuels produced as the main product in petroleum cracking operations, though the process may also be applied to analogous fractions of similar boiling range produced in the distillation of other types of hydrocarbonaceous materials or to various motor fuel blends comprising stocks from different sources.

More specifically, the invention is concerned with a method of treatment which results in the stabilization of various types of gasolines which have a tendency to deteriorate on storage with loss in such valuable properties as light color, low gum content and antiknock value, the deterioration being due principally to the action of oxygen and being accelerated by the photochemical effects of sunlight.

As a rule, little trouble is experienced in loss of the above mentioned properties during the storage of straight run gasolines, since there are substantially no olefins in the lower boiling fractions of crude oils, though tests indicate that higher molecular weight olefins may be present in the higher boiling fractions. The cracking process, however, which is employed to produce additional yields of gasoline from gas oils and petroleum residua invariably produces definite yields of unsaturated aliphatic hydrocarbons which have varying degrees of stability depending upon the type of unsaturation which characterizes them. The mono olefins are essentially stable even in direct contact with air and sunlight. Conjugated diolefins, however, such as butadiene and its derivatives, which are present in cracked gasolines produced under intensive cracking conditions, have been shown to be the compounds which first add oxygen to produce derivatives of a peroxidic character which in turn act autocatalytically to cause further oxygen addition with the development of gummy materials, compounds causing color and haze and ultimately definite amounts of acids, aldehydes, ketones and other oxygen-containing compounds.

The art of using inhibitors to retard the reactions of deterioration occurring in unstable gasoline has been developed to a considerable extent, and has largely overcome the disadvantages inherent in the chemical treatments aimed at stabilization, which entailed both loss of material and loss in antiknock rating. Use has been made of a wide variety of materials including both pure compounds and mixtures, and apparently the materials represent a large number of different chemical classes. They all, however,

they either preferentially absorb oxygen and prevent the initial formation of olefinic peroxides or that they decompose the peroxides initially formed so that the reactions of deterioration are halted for a period of time depending upon the amount and potency of the inhibitor. The present invention is a contribution to the inhibitor art and consists in the use of a particularly efficient class of blended materials as inhibitors in unstable hydrocarbon mixtures, particularly motor fuels.

In one specific embodiment, the present invention comprises the treatment of unstable cracked gasolines to preserve their valuable properties in respect to gum content, color and antiknock value with alcoholic solutions of alkyl-substituted para aminophenols and alkyl-substituted paraphenylenediamines.

An extensive series of investigations has indicated that solutions of the above character are particularly efficient in inhibiting the deterioration of cracked gasolines and that they are furthermore readily dispersed and dissolved when added in the relatively small quantities which have been found to be necessary for the proper protection of gasoline. The invention is therefore a definite contribution to the inhibitor art from two very practical standpoints, (1) that of furnishing inhibitors of high potency, and (2) that of furnishing a liquid material which is readily handled and quickly dissolved.

The general formulas of the two classes of compounds which are dissolved in alcohol in varying proportions to form the present type of inhibitors are given below, in which R represents alkyl-substituting groups and the other letters have their usual chemical significance.



Monoalkyl p-aminophenols      Dialkylphenylene diamines

R may represent methyl, ethyl, propyl, butyl, amyl, hexyl and other higher molecular weight aliphatic residues, and includes the isomeric forms. For example, mixtures of monomethyl p-aminophenol and dimethyl p-phenylenediamine may be dissolved in a suitable alcohol or mixtures may be made of compounds in which the substituting groups are different or absent in one of the compounds. An example of mixed

substituted compounds might be monoethyl p-aminophenol and p-phenylenediamine or mono-isoamyl p-aminophenol and either p-phenylenediamine di-isoamyl p-phenylenediamine. Obviously, by varying the character of the alkyl-substituting groups in the main classes of compounds and also the proportions thereof, a large number of alternative combinations are possible, which, however, will not have exactly the same inhibiting efficiency in a given unstable gasoline or the same comparative efficiency in different gasoline, so that various combinations are not exact equivalents. Furthermore, different compounds which are proposed as inhibitors will have different solubilities in different alcohols and blends thereof so that the amount of solvent necessary for making a sufficiently fluid inhibitor and assisting its dispersion throughout a large body of gasoline will also vary. Also either or both of the classes of compounds referred to may be treated in accordance with the invention.

It is particularly to be noted that all of the members of the two classes of substituted compounds whose single or joint use is proposed as inhibitors are solids at ordinary temperatures and as such are difficult to handle and difficult to dissolve in gasolines requiring inhibitors. The discovery that these compounds which have high inhibiting potency when properly dispersed through a body of gasoline could be easily handled and quickly dissolved when utilized in alcoholic solution is one of the notable contributions to the inhibitor art which characterizes the present invention. The various alcohols which may be used, which comprise usually the lower molecular weight aliphatic alcohols, have different solvent action upon different members of the classes proposed. The following table is introduced to indicate the relative solvent activity of a limited number of alcohols on a particular mixture of compounds from the two classes already mentioned which consisted of about 80% by weight of mono iso amyl p-aminophenol and 20% by weight of di-iso amyl p-phenylenediamine. The table shows the parts of solvent to one part by weight of the blend of compounds and indicates also whether a gasoline to which the solution was added in the concentration of 0.004% remained perfectly clear or precipitated out a small quantity of insoluble material. Incidentally the table also shows the corresponding induction periods of the gasoline to which the inhibitors were added, this figure indicating the time to measurable oxygen absorption in the standard bomb test:

#### Solvent action of alcohols

| Solvent                   | Parts of solvent to 1 part of solid | Condition of gasoline | Induction period, minutes |
|---------------------------|-------------------------------------|-----------------------|---------------------------|
| Methyl alcohol, absolute. | 1                                   | Cloudy                | 325                       |
|                           | 2                                   | Slightly cloudy       | 325                       |
|                           | 5                                   | Cloudy                | 330                       |
| Ethyl alcohol, absolute.  | 1                                   | Clear                 | 345                       |
|                           | 2                                   | do                    | 350                       |
|                           | 5                                   | do                    | 355                       |
| Butyl alcohol             | 1                                   | do                    | 335                       |
|                           | 2                                   | do                    | 350                       |
|                           | 5                                   | do                    | 360                       |
| Isobutyl alcohol          | 1                                   | do                    | 340                       |
|                           | 2                                   | do                    | 330                       |
|                           | 5                                   | do                    | 345                       |

The above table indicates that generally in the case of the solid combination employed, the solvent action of the aliphatic alcohols increased with increasing molecular weight, though the in-

duction period did not vary to any great extent. When the gasoline was cloudy or hazy after the addition of the inhibitor blend, it eventually separated some slight precipitate.

The following table is introduced to show further results when using different alcohols as solvents and when employing the same inhibiting materials in concentrations of 0.025% by weight of an unstable gasoline, which is an entirely practical percentage from the standpoint of cost, clarity of gasoline, color, drop, etc. One part by weight of the same mixture used when obtaining figures in the preceding table was dissolved in three parts by weight of the alcohol shown.

#### Effect of solvents on induction period

| Solvents           | Induction period, minutes | 20 |
|--------------------|---------------------------|----|
| Methyl alcohol     | 930                       |    |
| Ethyl alcohol      | 905                       |    |
| Propyl alcohol     | 980                       |    |
| Isopropyl alcohol  | 935                       |    |
| n-Butyl alcohol    | 1125                      |    |
| i-Butyl alcohol    | 1075                      | 25 |
| Sec. butyl alcohol | 1245                      |    |

In the following specific example which is introduced to show a very practical application of the present type of inhibitor to the treatment of an unstable gasoline, a blend of alcohols was used which apparently has a particularly good solvent action on the isoamyl derivatives mentioned as well as on other combinations of other compounds. The example is introduced to show the practical character of the process but is not intended to unduly limit the scope of the invention.

The blend of alcohols used consisted of 20% by volume of isobutyl alcohol with 80% by volume of absolute methyl alcohol. This blend dissolved an equal part by weight of a mixture which was substantially 80% mono iso amyl p-aminophenol and 20% di-iso amyl p-phenylenediamine. The solution was perfectly clear and could be added to test gasolines in amounts up to 0.1% without encountering difficulties in undue loss of color or the development of haze or undesirable precipitation. The cold test of the 1:1 blend of inhibiting solids and alcohol solvent was below -60° F. and the induction period of the gasoline to which it was added in an amount equivalent to 0.025% was raised from 150 minutes to 650 minutes. The advantage of using this particular blend can be seen from the fact that the methyl alcohol is considerably cheaper than the iso butyl alcohol.

The foregoing specification disclosing the character of the invention will enable those skilled in the art to which it pertains to approach its commercial value and the data introduced will show the type of results obtainable in practice, though neither section is intended to be unduly limiting.

I claim as my invention:

1. A method for stabilizing cracked gasoline against deterioration which comprises adding to the gasoline an alkyl-substituted para-aminophenol and an alkyl-substituted paraphenylenediamine dissolved in an alcoholic solvent comprising a butyl alcohol.

2. A method for stabilizing cracked gasoline against deterioration which comprises adding to the gasoline an alkyl-substituted para-aminophenol and an alkyl-substituted paraphenyl-

- enediamine dissolved in an alcoholic solvent comprising isobutyl alcohol.
3. A method for stabilizing cracked gasoline against deterioration which comprises adding to the gasoline a mixture of methyl and isobutyl alcohols having dissolved therein an alkyl-substituted para-aminophenol and an alkyl-substituted paraphenylenediamine.
4. An inhibitor for cracked gasoline comprising an alkyl-substituted para-aminophenol and an alkyl-substituted paraphenylenediamine dissolved in an alcoholic solvent comprising a butyl alcohol.
5. An inhibitor for cracked gasoline comprising an alkyl-substituted para-aminophenol and an alkyl-substituted paraphenylenediamine dissolved in an alcoholic solvent comprising isobutyl alcohol.
6. An inhibitor for cracked gasoline comprising a mixture of methyl and isobutyl alcohols having dissolved therein an alkyl-substituted para-aminophenol and an alkyl-substituted paraphenylenediamine.
7. A method for stabilizing cracked gasoline against deterioration which comprises adding to the gasoline a relatively small amount of a solution of an alkyl-substituted para-aminophenol and an alkyl-substituted paraphenylenediamine, the first-named compound being in substantially greater proportion than the second, and the solvent of said solution comprising a major proportion of methyl alcohol and a minor proportion of an aliphatic alcohol having from 2 to 4 carbon atoms.
8. A method for stabilizing cracked gasoline against deterioration which comprises adding to the gasoline a relatively small amount of a solution of mono-iso-amyl para-aminophenol and di-iso-amyl paraphenylenediamine, the first-named compound being in substantially greater proportion than the second, and the solvent of said solution comprising a major proportion of methyl alcohol and a minor proportion of an aliphatic alcohol having from 2 to 4 carbon atoms.
9. A method for stabilizing cracked gasoline against deterioration which comprises adding to the gasoline a relatively small amount of a solution of an alkyl-substituted para-aminophenol and an alkyl-substituted paraphenylenediamine, the first-named compound being in substantially greater proportion than the second, and the solvent of said solution comprising a major proportion of methyl alcohol and a minor proportion of a butyl alcohol.
10. A method for stabilizing cracked gasoline against deterioration which comprises adding to the gasoline a relatively small amount of a solution of mono-iso-amyl para-aminophenol and di-
- iso-amyl paraphenylenediamine, the first-named compound being in substantially greater proportion than the second, and the solvent of said solution comprising a major proportion of methyl alcohol and a minor proportion of a butyl alcohol.
11. An inhibitor for cracked gasoline comprising a solution of an alkyl-substituted para-aminophenol and an alkyl-substituted paraphenylenediamine, the first-named compound being in substantially greater proportion than the second, and the solvent of said solution comprising a major proportion of methyl alcohol and a minor proportion of an aliphatic alcohol having from 2 to 4 carbon atoms.
12. An inhibitor for cracked gasoline comprising a solution of mono-iso-amyl para-aminophenol and di-iso-amyl paraphenylenediamine, the first-named compound being in substantially greater proportion than the second, and the solvent of said solution comprising a major proportion of methyl alcohol and a minor proportion of an aliphatic alcohol having from 2 to 4 carbon atoms.
13. An inhibitor for cracked gasoline comprising a solution of an alkyl-substituted para-aminophenol and an alkyl-substituted paraphenylenediamine, the first-named compound being in substantially greater proportion than the second, and the solvent of said solution comprising a major proportion of methyl alcohol and a minor proportion of a butyl alcohol.
14. An inhibitor for cracked gasoline comprising a solution of mono-iso-amyl para-aminophenol and di-iso-amyl paraphenylenediamine, the first-named compound being in substantially greater proportion than the second, and the solvent of said solution comprising a major proportion of methyl alcohol and a minor proportion of a butyl alcohol.
15. A method for stabilizing cracked gasoline against deterioration which comprises adding to the gasoline a relatively small amount of a solution of an alkyl-substituted para-aminophenol and an alkyl-substituted paraphenylenediamine, the first-named compound being in substantially greater proportion than the second, and the solvent of said solution comprising a major proportion of a mixture of methyl alcohol and an aliphatic alcohol having from 2 to 4 carbon atoms.
16. An inhibitor for cracked gasoline comprising a solution of an alkyl-substituted para-aminophenol and an alkyl-substituted paraphenylenediamine, the first-named compound being in substantially greater proportion than the second, and the solvent of said solution comprising a major proportion of a mixture of methyl alcohol and an aliphatic alcohol having from 2 to 4 carbon atoms.

CHARLES G. DRYER.